

## UNITED STATES PATENT OFFICE

2,098,567

METHOD OF INCORPORATING NITROGEN  
IN ALLOY STEELS

George F. Comstock and Viatcheslav V. Efimoff,  
Niagara Falls, N. Y., assignors to The Titanium  
Alloy Manufacturing Company, New York,  
N. Y., a corporation of Maine

No Drawing. Application July 30, 1937,  
Serial No. 156,520

20 Claims. (Cl. 75—127)

Our invention relates more particularly to improved methods of introducing nitrogen into alloy steels having a high chromium content to improve their physical properties.

5 It is well-known that cast high-chromium steels as ordinarily produced consist of rather coarse crystals that result in weakness, and can not be refined by heat-treatment, and one of the 10 objects of our invention is to devise improved and simplified methods to refine the grain of such steels without incurring the unsoundness which often results from the addition of nitrogen, or requiring the superheating of the finished steel which is likely not only to create difficulties in 15 maintaining the furnace structure but also in preserving the desired steel composition.

Our invention consists, therefore, in new and improved methods for adding nitrogen to high chromium or other steels, in which nitrogen has 20 been shown to have beneficial effects such as reducing the grain size and improving the mechanical properties.

Nitrogen has been added to these steels up to the present time chiefly as high-nitrogen ferro-chromium. Although this method with proper 25 precautions may be used successfully for obtaining the desired improvement in the properties of the steel, it is subject to certain limitations which interfere seriously with its use in many steel plants.

One of these difficulties is the necessity for superheating the molten steel for a considerable period of time after the addition of high-nitrogen ferrochromium, and this practice is harmful 35 to the furnace refractories and also apt to alter the composition of the steel from that which it is desired to make, besides adding to the expense by requiring longer operation of the furnace.

Another difficulty is the prevalence of gas 40 holes or porosity in the castings made from steel in which high-nitrogen ferrochromium has been used. This trouble has been so serious in some foundries that the use of high-nitrogen ferrochromium was entirely abandoned.

45 In the course of our experiments and tests in melting and casting high-chromium steels, we have discovered that when titanium cyanonitride (TiCN) or zirconium cyanonitride (ZrCN) is used as the source of nitrogen for incorporating nitrogen in them, the advantages of grain refinement and improved mechanical properties are obtained without the necessity for superheating the melt, and without unsoundness in the castings.

50 The incorporation of titanium or zirconium

cyanonitride in these steels is not attended with any difficulty, and is as simple as the addition of any other alloying ingredient. The former compound, (TiCN), as regularly produced for this and other uses by methods described by William M. Thornton Jr. in his book on "Titanium" published in 1927 by Chemical Catalog Company of New York, N. Y., page 53 contains over 75% titanium and less than 5% carbon, iron, silicon or other impurities, with about 10 to 20% of 10 nitrogen.

A representative analysis of such titanium cyanonitride is as follows:

|                         | Per cent |    |
|-------------------------|----------|----|
| Titanium                | 80.04    | 15 |
| Carbon                  | 3.06     |    |
| Iron                    | 1.94     |    |
| Silicon                 | 0.29     |    |
| Nitrogen and impurities | 14.67    |    |
|                         |          | 20 |
|                         | 100.00   |    |

Such alloy is a hard but rather brittle substance, and differs from titanium carbide in being more easily crushable to any size desired for adding to molten steel.

Zirconium cyanonitride, as produced by methods set forth in United States Letters Patent to Barton No. 1,351,091 of August 31, 1920, however, is a somewhat softer and more easily crushed compound, and is perhaps slightly less desirable for the purposes of our invention, since its nitrogen content is lower and more of it therefore must be used. It is also more easily burned and lost by oxidation than titanium cyanonitride. A representative analysis is as follows:—

|                         | Per cent |    |
|-------------------------|----------|----|
| Zirconium               | 84.0     |    |
| Carbon                  | 3.0      | 40 |
| Silicon                 | 2.0      |    |
| Titanium                | 0.2      |    |
| Iron                    | 0.1      |    |
| Nitrogen and impurities | 10.7     |    |
|                         |          | 45 |
|                         | 100.0    |    |

Although the following exposition of the advantages of our invention and description of our improved methods refers chiefly to titanium cyanonitride which in some ways may be more desirable and practical to use, it should be understood that the invention applies with equal force to the use of the similar compound of zirconium.

A further advantage derived from the employment of our new methods for adding nitrogen to

high-chromium or other steels results from the action of the titanium which accompanies the nitrogen in the titanium cyanonitride. The practicability of our methods depends, of course, 5 on the higher affinity of chromium than titanium for nitrogen. In passing from its combination with titanium into the chromium steel, the nitrogen leaves the titanium, with which it had been combined, free to exert the usual beneficial effects 10 of titanium as a deoxidizer and scavenger, thereby improving the cleanliness and soundness of the finished steel.

Evidence of such action is afforded by the recoveries of nitrogen and titanium observed when 15 titanium cyanonitride has been used in various ways in chromium steels. With nitrogen recoveries of 19 to 68% from this compound, the titanium recoveries in the steel were only from about 3 to 11%, thereby showing that titanium 20 was released from combination with nitrogen and passed out of the steel. Since titanium is known not to be volatile at steel-making temperatures, such titanium must have been eliminated as the oxide, and therefore has acted to deoxidize the 25 steel without leaving any appreciable titanium content in the resulting steel.

As an example of the use of titanium cyanonitride instead of high-nitrogen ferrochromium as the source of nitrogen in high-chromium steels, 30 the following tests which we have made will now be described.

The materials indicated in the following table were melted in a magnesia crucible by heating with an Ajax-Northrup high-frequency induction 35 furnace, the time for melting being about the same for each heat, with the contents of each heat being poured into a single mold when at temperatures of about 2810° F. No superheating was applied to any of the melts. The titanium 40 cyanonitride, ground to 20 mesh and finer, was mixed with the low-carbon ferrochromium in Heat 2, and both were added together after the iron scrap was fused.

After the ingots had solidified, their top ends 45 were nicked and broken to examine the fractures, and the grain size was estimated by counting the number of crystal facets observed within a one-inch length at several places on the fracture.

50 The average result, together with a note on the soundness of the fracture, is now given for each heat in the following table.

|    |                                   | Heat No. |        |          |
|----|-----------------------------------|----------|--------|----------|
|    |                                   | 1        | 2      | 3        |
| 55 | Pure iron scrap, lbs.             | 10.5     | 10.5   | 11       |
|    | High-carbon ferrochromium, lbs.   | 0.25     | 0.25   | 0.25     |
|    | Low-carbon ferrochromium, lbs.    | 5.75     | 5.75   | 0        |
|    | High-nitrogen ferrochromium, lbs. | 0        | 0      | 5.5      |
|    | Titanium cyanonitride, gms.       | 0        | 300    | 0        |
| 60 | Low-carbon ferromanganese, gms.   | 20       | 20     | 20       |
|    | 50% ferrosilicon, gms.            | 35       | 35     | 35       |
|    | Per cent nitrogen added           | 0        | 0.44   | 0.23     |
|    | Average grain-size, inches.       | 0.72     | 0.09   | 0.06     |
|    | Shape of riser surface            | Shrunk   | Shrunk | Expanded |
|    | Soundness of fracture             | Good     | Good   | Unsound  |

65 Our invention is of course applicable to other methods of melting than the one described in the above example, and the titanium cyanonitride may also be added to the steel in other ways than the one described without departing 70 from the essential features of our invention. For example, when making 25% chromium steel in an acid electric furnace of the direct arc type, the titanium cyanonitride was added to the molten iron scrap and covered immediately with low-carbon ferrochromium, and similar results re-

garding soundness and grain-size of the castings were obtained as we have hereinbefore described in detail.

The titanium cyanonitride may also be added just before the iron scrap is completely melted, 5 or even stirred into the completed melt after the ferrochromium, although adding it either directly before or with the ferrochromium is the preferred practice. The addition of TiCN should be made in the furnace rather than in the ladle, 10 since this compound is too refractory to mix well with the steel in the short time available in the ladle, and the reaction involving the liberation of nitrogen also requires a reasonable time.

For the best recovery of nitrogen the presence 15 of some slag which will absorb titanium dioxide is desirable, so that in induction furnace melting where there may be very little slag on the melt, the addition of a small amount of lime we have found to be desirable when titanium cyanonitride is used as a source of nitrogen for grain refinement of chromium steels.

In using zirconium cyanonitride by the method of our invention, exactly the same procedure was carried out as described for Heat No. 2 of the 25 previous example given in respect to titanium cyanonitride, except that a smaller charge was used (15 pounds instead of 17 pounds) and 175 grams of zirconium cyanonitride were substituted for the titanium cyanonitride. This involved an 30 addition of 0.28% nitrogen, and gave a good sound ingot with an average grain size of about 0.17 inch, decidedly finer than the untreated steel. Zirconium, which is liberated in the steel to which our invention is applied in the same way 35 as has been explained for titanium, has a similar effect in deoxidizing and improving the soundness of the steel, so that the results of the invention are equally beneficial no matter whether titanium cyanonitride, or the closely related compound 40 zirconium cyanonitride, is used.

Our invention may also be applied to other kinds of steel than the plain chromium steel mentioned above, such as steels containing both 45 chromium and nickel, or other alloying elements, in which a fine grain-size, and absence of gas cavities, are desired. The tensile properties in the resulting steels are substantially those which would be expected from the nitrogen contents.

We claim as our invention:

1. A method of incorporating nitrogen in alloy 55 steels which consists in adding a cyanonitride of an element chosen from the group consisting of titanium and zirconium as an alloy to the other ingredients to form the steel.

2. A method of incorporating nitrogen in chromium steels which consists in adding a cyanonitride of an element chosen from the group consisting of titanium and zirconium as an alloy to the other 60 ingredients to form the steel.

3. A method of incorporating nitrogen in alloy steels which consists in adding titanium cyanonitride as an alloy to the other ingredients to form the steel.

4. A method of incorporating nitrogen in chromium steels which consists in adding titanium cyanonitride as an alloy to the other ingredients to form the steel.

5. A method of incorporating nitrogen in high-chromium steel castings which consists in adding titanium cyanonitride as an alloy to the other ingredients to form the steel.

6. A method of incorporating nitrogen in alloy steels which consists in adding zirconium cyanonitride as an alloy to the other ingredients to form the steel.

- nitride as an alloy to the other ingredients to form the steel.
7. A method of incorporating nitrogen in chromium steels which consists in adding zirconium cyanonitride as an alloy to the other ingredients to form the steel.
8. A method of incorporating nitrogen in high-chromium steel castings which consists in adding zirconium cyanonitride as an alloy to the other ingredients to form the steel.
9. A method of incorporating nitrogen in chromium steels which consists in adding titanium cyanonitride and low-carbon ferrochromium to the steel-forming ingredients before melting the charge to produce the steel.
10. A method of incorporating nitrogen in chromium steels which consists in adding titanium cyanonitride and low-carbon ferrochromium to the molten steel-forming ingredients.
11. In the method of making chromium steel containing nitrogen, the step which consists in adding to the steel forming ingredients titanium cyanonitride before melting.
12. In the method of making chromium steel containing nitrogen, the steps which consist in adding to the steel forming ingredients including iron and scrap titanium cyanonitride after the iron scrap has melted, and then adding ferrochromium to the melt.
13. In the method of making chromium steel containing nitrogen, the steps which consist in adding to the molten steel-forming ingredients titanium cyanonitride, and then stirring the molten mass.
14. In the method of making chromium steel containing nitrogen, the steps which consist in adding to the molten steel-forming ingredients ferrochromium mixed with titanium cyanonitride, and then stirring the molten mass.
15. In the method of making chromium steel containing nitrogen, the steps which consist in adding to the molten steel-forming ingredients in the furnace titanium cyanonitride, and then stirring the molten mass.
16. In the method of making chromium steel containing nitrogen, the steps which consist in adding to the molten steel-forming ingredients in the furnace ferrochromium mixed with titanium cyanonitride, and then stirring the molten mass.
17. In the method of making chromium steel containing nitrogen, the step which consists in adding titanium cyanonitride as an alloy to the other ingredients to form such steel, the nitrogen acting to refine the grain size with the titanium deoxidizing and degasifying the steel.
18. A method of incorporating nitrogen in chromium steel which comprises adding to the molten steel-forming ingredients titanium cyanonitride, and also lime to form a slag to absorb the titanium dioxide produced in the molten mass.
19. A method of incorporating nitrogen in chromium steel which comprises adding to the molten steel-forming ingredients ferrochromium mixed with titanium cyanonitride, and also lime to form a slag to absorb the titanium dioxide produced in the molten mass.
20. In the method of making chromium steel containing nitrogen, the step which consists in adding to the steel forming ingredients zirconium cyanonitride before melting.

25

30

35

GEORGE F. COMSTOCK.  
VIATCHESLAV V. EFIMOFF.